# EUROPEAN PATENT SPECIFICATION

(11) **EP 0 250 116 B1**
(45) Date of publication and mention of the grant of the patent: **04.03.1992**
(21) Application number: 87304817.7
(22) Date of filing: 01.06.1987
(51) Int. Cl.: C10C 3/00, D01F 9/12

(54) **Pressure settling of mesophase pitch**
Druckablagerung von mesophasem Pech
Précipitation à pression de brai à mésophase

(30) Priority: 09.06.1986 US 871978
(43) Date of publication of application: 23.12.1987
(73) Proprietor: CONOCO INC., Ponca City Oklahoma 74603 (US)
(72) Inventor: Romine, Hugh Ernest, Ponca City Oklahoma 74604 (US)
(74) Representative: Woodman, Derek

(56) References cited:
- EP-A- 0 044 714
- EP-A- 0 055 024
- EP-A- 0 087 301
- EP-A- 0 089 840
- EP-A- 0 090 637
- FR-A- 2 549 486
- US-A- 4 529 499

## Description

This invention relates to production of mesophase pitch suitable for manufacture of carbon fibers and other carbon artifacts. More particularly, the invention is directed to an improved settling process for separating mesophase pitch from a heat soaked heavy aromatic hydrocarbon feedstock.

There has been a substantial effort in recent years to produce anisotropic pitch comprised of from 40 to 100 percent mesophase, which can then be spun into carbon fibers. One approach to production of mesophase involves heat soaking a heavy aromatic hydrocarbon feedstock at conditions such that a more dense mesophase material forms. Variations of the heat soaking process include sparging inert gas through the feedstock during heat soaking, agitating the feedstock during heat soaking, or a combination of sparging and agitation, as described in U.S. Patent 4,209,500 to Chwastiak.

U.S. Patent 4,317,809 to Lewis et al describes heat soaking a mesophase precursor material at high pressure, followed by additional heat soaking at atmospheric pressure with gas sparging.

U.S. Patent 4,454,020 to Izumi et al describes heat soaking mesophase precursor material, separating a heavier anisotropic phase, and further heating the separated portion.

EP-A- 44,714 describes a basic heat soak and gravity separation process for producing mesophase pitch which involves cooling the heat soaked material enough to stop boiling so that settling of mesophase pitch readily occurs.

Many other descriptions of variations of the heat soaking procedure for producing mesophase appear in the literature, and the present invention is applicable in general to any process in which a mesophage forming feedstock is heat soaked to form mesophase and the thus formed mesophase recovered from the heat soaked feedstock. Specific mesophase-forming conditions of temperature, heat soaking time, feedstock composition, gas sparging, agitation and the like have been extensively developed in the prior art, and are not a part of the present invention, as the present invention is generally applicable in any case where a mesophage-forming feedstock is heat soaked and mesophase pitch recovered therefrom, without regard to the specific conditions under which the mesophase is formed.

### Summary of the Invention

According to the present invention, mesophase pitch is recovered from a heat soaked mesophase precursor feedstock by applying a pressure higher than the heat soaking pressure to the heat soaked material, allowing more dense mesophase material to settle by gravity, and separating the settled material from the less dense heat soaked material.

The settling temperature can be the same as or lower than the heat soaking temperature, but should not be low enough that increased viscosity substantially impedes settling.

During the heat soaking stage, the feedstock undergoes cracking reactions leading to production of mesophase and other components, including gaseous components. These gaseous cracking components continue to evolve during the settling step, if settling is conducted at or near the heat soaking temperature, resulting in agitation of the material to be settled.

EP-A- 44,714, referred to earlier attempts to overcome this problem by cooling the heat soaked material to reduce gas evolution from cracking, as well as boiling of the material, such that settling is not hindered by gas movement through the settling material. This technique is subject to the drawback of increased viscosity with decreasing temperature, such that the time required for settling is increased.

According to the present invention, an increased pressure is applied to the heat soaked material, sufficient to prevent or réduce boiling and to substantially maintain cracked gaseous components in solution, such that the settling occurs without the necessity of a viscosity-increasing cooling step.

In consequence of our invention, we are able to provide a process for rapidly settling mesophase pitch form heat soaked mesophase precursor, and to provide a process for controlling certain characteristics of mesophase pitch which is separated from a heat soaked mesophase precursor.

The invention will no be more particularly described with reference to the accompanying drawings, which are by way of example only and in which:

Figure 1 is a schematic flowchart showing a batch type process in accordance with the invention.

Figure 2 is a schematic flowchart showing a continuous type process in accordance with the invention.

Figure 3 is a schematic flowchart showing another variation of a continuous type process in accordance with the invention.

The term "mesophase" as used herein refers to an optically anisotropic material formed by any of several variations of a process in which a heavy aromatic hydrocarbon feedstock is heat soaked at conditions known in the art to produce a substantial amount of the optically anisotropic mesophase material.

Heavy aromatic hydrocarbon feedstocks suitable for formation of mesophase are also known in the art, and include, among others, petroleum pitch, decant oil and thermal tar.

A basic batch type version of the process of the invention is illustrated in Figure 1, where heavy aromatic hydrocarbon feedstock from tank 10 is pumped to heat soak vessel 12 where it is heated by any suitable means (not shown) until a substantial amount of mesophase has formed. During all or part of the heating, an inert sparge gas from line 14 may be sparged through the feedstock to remove lighter hydrocarbon components and to effect more efficient heat transfer. The sparging gas exits through line 16.

When the heat soak is completed, flow of sparging gas is stopped, the soak tank 12 is sealed, and soak tank 12 is then pressurized by gas from cylinder 18 to a pressure sufficient to prevent boiling of the contents and to maintain cracked gases in solution. With the system closed in and no appreciable gas movement through the heat soaked material, the more dense mesophase readily settles to the bottom of tank 12, and is withdrawn through mesophase recovery line 20.

A basic continuous type version of the process of the invention is illustrated in Figure 2, where feedstock from tank 30 is heated in heater 32 and passed to distillation or flash tower 34. The tower bottoms are fed through line 36 to soak tank 38, and sparge gas may be passed through the soak tank 38 via lines 40 and 42. If sparge gas is not used, vapors from tank 38 may be returned to tower 34 via line 44. Soak tank 38 may have internal baffles (not shown) or other flow control means to assure uniform residence time of the feedstock in tank 38. The heat soaked material from soak tank 38 is passed to settling tank 46 via line 48. Settling tank 46 may also include internals (not shown) to assure appropriate residence time and to direct settled mesophase to mesophase recovery line 50. The non-mesophase material may be removed from settling tank 46 via line 52, or recycled to soak tank 38 via line 54. An increased pressure in settling tank 46 may be maintained by gas pressure from gas cylinder 56.

A more elaborate continuous type version of the process of the invention in which two different mesophase products are recovered is illustrated in Figure 3. The system depicted in Figure 3 is similar to the Figure 2 version, but includes a second settling tank 60 which is fed with non-mesophase material from first settling tank 46 via line 62. Second settling tank 60 normally is maintained at a lower temperature and pressure than first settling tank 46. Pressure in tank 60 may be controlled with gas cylinder 64, and unsettled material may be returned to heater 32 via recycle line 66. Settled mesophase from tank 60 is recovered via line 68. Elements of Figure 3 which are common with Figure 2 have like identification numbers.

Temperature is an important variable during pressure settling due to the strong temperature dependence of the solubility of mesophase in isotropic heavy aromatic pitch. Decreased settling temperature increases the yield of mesophase while lowering its average molecular weight. Through proper temperature control, two distinct types of mesophase pitch or blends thereof can be isolated. Settling at or near the soaking temperature yields a relatively high melting, highly coalesced mesophase pitch. This material is almost entirely comprised of anisotropic mesophase. Subsequent cooling of the saturated heat soaked feedstock leads to precipitation and settling of "new" lower melting mesophase pitch which is less highly coalesced. This lower melting mesophase pitch is generally 50 to 90 weight percent anisotropic material.

Thus, the embodiment illustrated in Figure 3 enables a "tailoring" of mesophase product which is not possible in a single settling step operation.

The following example illustrates production of two mesophase pitch products having different properties using a process as described above in relation to Figure 3.

### Example

A flashed thermal tar feedstock is heated to about 460°C and passed to a flash tower maintained at about 375 kPa. The flash tower bottoms (deep flashed thermal tar) are passed to a heat soak tank maintained at about 375 kPa and about 440°C. Residence time of the deep flashed thermal tar in the heat soak tank is about six hours. Heat soaked thermal tar is pumped from the soak tank to a first settling tank maintained at about 620 kPa without substantial cooling of the heat soaked material. Residence time in the first settling tank is about ten minutes. The increased pressure essentially prevents boiling in the settling tank, and about 35 percent by volume of the heat soaked material settles out as "old" mesophase pitch which is essentially 100 percent anisotropic material having a melting point of about 450°C. Unsettled material from the first settling tank is passed to a second settling tank maintained at a pressure of 375 kPa and a temperature of about 250°C with a residence time of about twenty minutes. A "new" mesophase pitch in an amount of about 50 percent of the feed to the second settling tank, comprising about 75 percent anisotropic material and having a melting point of about 200°C, is recovered. Unsettled material from the second settling tank is recycled to the heater feed.

This example illustrates that high melting mesophase can be quickly settled from heat soaked feedstock using an increased pressure, and a low melting mesophase can be precipitated from the remaining saturated heat soaked material.

There are many variations and embodiments of the invention which will be apparent to those skilled in the art of making mesophase. Directionally, much is known as to the effects of varying such things as feedstock, soaking time and temperature, sparging, agitation, cooling of soaked feedstock, and the like. Soaking temperatures of from 350 to 475°C and soaking times of from 0.5 to 120 hours are generally considered to be the practical limits for the process, with shorter times within that range generally being used with temperatures nearer the higher limit. The conditions for a particular run may be influenced by factors such as time available, feedstock properties, equipment limitations, desired product properties, etc., as is known in the art. However, the prior art has not recognized that rapid settling can be effected by increasing pressure on a heat soaked mesophase-containing feedstock, and further has not recognized that rapid initial settling of mesophase, made possible by use of increased settling pressure, provides a capability for producing mesophase pitches having specific desired properties such as low melting point.

The feature which permeates all the embodiments of the invention is the use of an initial settling pressure greater than the pressure at which the feedstock was heat soaked. The heat soaking pressure can be higher, lower or equal to atmospheric pressure, and the settling pressure needs to be sufficiently higher than the soaking pressure to retard or eliminate boiling in the soak tank and to keep in solution any gases generated by cracking after the soaking is completed . A pressure as little as 30 kPa above the soaking pressure can be effective in some cases, and in other cases it may be desirable to use a pressure as much as 2 MPa higher than the soaking pressure.

## Claims

1. A process for producing mesophase pitch wherein a heavy aromatic hydrocarbon feedstock is heat soaked until a portion of the feedstock has been converted to optically anisotropic material,
the heat soaked material is subjected to a pressure higher than the pressure at which the heat soaking took place whereby boiling of the heat soaked material is reduced, gases formed by cracking of heat soaked material during settling are substantially maintained in solution, and settling of mesophase pitch is enhanced, and the mesophase pitch is recovered from the heat soaked material by gravity settling.

2. A process as claimed in claim 1 wherein said heat soaked material is retained in a heat soaking vessel, and the pressure in said vessel is increased prior to recovery of settled mesophase pitch therefrom.

3. A process as claimed in claim 1 wherein said heat soaked material is transferred from a heat soaking vessel to a settling vessel maintained at a higher pressure than said heat soaking vessel, and mesophase pitch is recovered from said settling vessel.

4. A process as claimed in claim 3 wherein the remaining heat soaked material in said settling vessel, after recovery of mesophase pitch therefrom, is returned to said heat soaking vessel and further heat soaked.

5. A process as claimed in claim 3 wherein the remaining heat soaked material in said settling vessel, after recovery of mesophase pitch therefrom, is transferred to a second settling vessel from which additional settled mesophase pitch is recovered.

6. A process as claimed in any of claims 1 to 5 which comprises
(a) heat soaking a heavy aromatic hydrocarbon feedstock at a temperature of from 350 to 475°C for a time of from 0.5 to 120 hours and at a first pressure until a substantial portion of said feedstock has been coverted to mesophase pitch;
(b) subjecting said heat soaked feedstock containing mesophase pitch to a pressure higher than said first pressure
(c) allowing mesophase pitch to settle from said heat soaked feedstock; and
(d) recovering said settled mesophase pitch.

## Revendications

1. Procédé de production d'un brai à mésophase, dans lequel une charge formée d'un hydrocarbure aromatique lourd est traitée par maturation à la chaleur jusqu'à ce qu'une portion de cette charge ait été convertie en matière optiquement anisotrope,
la matière traitée par maturation thermique est exposée à une pression supérieure à la pression à laquelle la maturation thermique a eu lieu de manière à réduire l'ébullition de la matière ayant subi la maturation thermique, les gaz formés par craquage de la matière traitée par maturation thermique pendant la sédimentation sont principalement maintenus en solution et la sédimentation du brai à mésophase est améliorée, et le brai à mésophase est recueilli par sédimentation par gravité de la matière traitée par maturation thermique.

2. Procédé suivant la revendication 1, dans lequel ladite matière traitée par maturation thermique est retenue dans le récipient de maturation thermique et la pression dans ce récipient est élevée avant que le brai à mésophase sédimenté n'en soit recueilli.

3. Procédé suivant la revendication 1, dans lequel la matière traitée par maturation thermique est transférée d'un récipient de maturation thermique à un récipient de sédimentation maintenu à une pression plus haute que dans le récipient de maturation thermique, et le brai à mésophase est recueilli du récipient de sédimentation.

4. Procédé suivant la revendication 3, dans lequel la quantité restante de matière traitée par maturation thermique dans ledit récipient de sédimentation, après que le brai à mésophase en a été recueilli, est recyclée au récipient de maturation thermique et la maturation thermique en est poursuivie.

5. Procédé suivant la revendication 3, dans lequel la matière traitée par maturation thermique restant dans le récipient de sédimentation, après que le brai à mésophase en a été recueilli, est transférée dans un second récipient de sédimentation duquel on recueille une quantité additionnelle de brai à mésophase sédimenté.

6. Procédé suivant l'une quelconque des revendications 1 à 5, qui consiste
(a) à effectuer la maturation thermique d'une charge hydrocarbonée aromatique lourde à une température allant de 350 à 475°C pendant une durée de 0,5 à 120 heures et à une première pression jusqu'à ce qu'une portion importante de ladite charge ait été convertie en brai à mésophase ;
(b) à soumettre ladite charge traitée par maturation thermique contenant le brai à mésophase à une pression supérieure à ladite première pression ;
(c) à laisser le brai à mésophase se séparer par sédimentation de la charge traitée par maturation thermique ; et
(d) à recueillir le brai à mésophase sédimenté.

## Patentansprüche

1. Verfahren zur Herstellung eines Mesophasenpechs, worin eine schwere aromatische Kohlenwasserstoffbeschickung mit Wärme durchdrungen bzw. durchsickert wird, bis ein Teil der Beschickung in optisch anisotropes Material umgewandelt worden ist,
das wärmedurchdrungene Material einem Druck ausgesetzt wird, der höher ist als der Druck, bei dem das Wärmedurchdringen stattgefunden hat, wodurch das Sieden des wärmedurchdrungenen Materials verringert wird, Gase, gebildet durch Cracken von wärmedurchdrungenem Material während des Absetzens, im wesentlichen in Lösung gehalten werden und das Absetzen des Mesophasenpechs verstärkt wird, und das Mesophasenpech aus dem wärmedurchdrungenen Material durch Schwerkraftabsetzen gewonnen wird.

2. Verfahren nach Anspruch 1, worin das wärmedurchdrungene Material in einem Wärmedurchdringbehälter gehalten wird und der Druck in dem Behälter vor der Gewinnung des abgesetzten Mesophasenpechs daraus erhöht wird.

3. Verfahren nach Anspruch 1, worin das wärmedurchdrungene Material aus einem Wärmedurchdringbehälter in einen Absetzbehälter, der bei einem höheren Druck als der Wärmedurchdringbehälter gehalten wird, übertragen wird und Mesophasenpech aus dem Absetzbehälter gewonnen wird.

4. Verfahren nach Anspruch 3, worin das verbleibende wärmedurchdrungene Material in dem Absetzbehälter nach dem Gewinnen von Mesophasenpech daraus in den Wärmedurchdringbehälter rückgeführt und weiter wärmedurchdrungen wird.

5. Verfahren nach Anspruch 3, worin das verbleibende wärmedurchdrungene Material in dem Absetzbehälter nach dem Gewinnen von Mesophasenpech daraus in einen zweiten Absetzbehälter überführt wird, aus dem zusätzlich abgesetztes Mesophasenpech gewonnen wird.

6. Verfahren nach einem der Ansprüche 1 bis 5, das
(a) das Wärmedurchdringen einer schweren aromatischen Kohlenwasserstoffbeschickung bei einer Temperatur von 350 bis 475 C über eine Zeit von 0,5 bis 120 Stunden und bei einem ersten Druck, bis ein wesentlicher Teil der Beschickung in Mesophasenpech umgewandelt worden ist;
(b) das Aussetzen der wärmedurchdrungenen Beschickung, enthaltend Mesophasenpech, einem Druck, der höher ist als der erste Druck,
(c) das Absetzenlassen von Mesophasenpech aus der wärmedurchdrungenen Beschickung und
(d) das Gewinnen von abgesetztem Mesophasenpech umfaßt.
